

## UNITED STATES PATENT OFFICE

2,326,028

## SPARKING PLUG ELECTRODE

William Thomas Griffiths, Battledown, Cheltenham, England, assignor to The International Nickel Company, Inc., New York, N. Y., a company of Delaware

No Drawing. Application May 27, 1942, Serial No. 444,745. In Great Britain January 31, 1941

2 Claims. (Cl. 123—169)

This invention relates to sparking plugs for internal combustion engines. In internal combustion engines of high efficiency, such as those used in aeroplanes, the sparking plugs often have electrodes of precious metal. As a rule, alloys of platinum, such as those with iridium, rhodium and the like, are used and are made from metals having the purity generally available commercially at the present time.

It has been found that sparking plugs made from such alloys are liable to fail in service under severe operating conditions, so that their life is not as long as it might be. The primary object of this invention is to overcome this drawback.

It is an object of this invention to provide an improved sparking plug electrode having a longer life than those now used commercially.

It is a further object of this invention to provide an improved platinum-rhodium sparking plug electrode.

I have found that in order that the electrodes shall give the best service, in particular prolonged life, under severe working conditions, it is of the utmost importance that the alloys from which the electrodes are made should be as nearly as possible free from impurities which would produce embrittlement, either alone or with any other element or elements contained in the alloy or taken up by it in service. This is surprising because the total amount of impurities present in precious metals used for this purpose at present is so small that it would not be expected that they would have any effect at all upon electrodes made from the precious metals. I have found, however, that the elements platinum, rhodium, iridium and osmium in the forms in which they are normally available commercially contain enough impurities to shorten the life of an electrode made from them. An alloy which is often used is that consisting of about 90% platinum and about 10% rhodium, and it has now been found that commercial rhodium introduces tellurium and bismuth into the alloy in harmful amounts.

In my invention I make the electrodes from one of the metals platinum, rhodium, iridium and osmium, or an alloy of one or more of these, containing so little of any element or elements which, even in a small quantity, would produce embrittlement that the presence of such an element or elements cannot in general be determined with certainty by the usual methods of chemical analysis but only spectrographically or microchemically. In any case the total amount

of such an element or elements in the metal or alloy does not exceed about 0.01%, and preferably it is less than about 0.005%.

As has been indicated above, in alloys containing rhodium the principal elements that may not be present in more than the amounts given above are tellurium and bismuth. Thus the presence of as little as 0.003% tellurium and 0.003% bismuth may shorten the life of an electrode made from 10% rhodium and 90% platinum. These tellurium and bismuth contents are normally introduced into the alloys as impurities of the rhodium. I have found that increased life may be obtained by employing platinum free from tellurium and bismuth together with rhodium containing 0.005% bismuth (as determined by spectrographic analysis) and 0.024% tellurium (as determined microchemically). Then in the alloy containing 90% platinum and 10% rhodium the tellurium and bismuth contents are 0.0024% and 0.0005% respectively, making about 0.003% in all. Naturally the purer the alloy, the longer the life that the electrode is likely to have. Other elements besides tellurium and bismuth which may produce embrittlement and which may constitute impurities in the precious metals commercially available are the other elements of the sulphur group (sulphur and selenium), the other elements of the phosphorus group (phosphorus, arsenic and antimony), lead, tin and silicon. Of course, in the example given above care is taken that these other embrittlement producing elements are either completely absent or present at the most in amounts that cannot be determined by ordinary chemical analysis.

In producing electrodes according to the invention the precious metals in question must in general be re-refined before the alloys are made, that is to say, the commercial metals are treated to reduce any impurities to amounts which are capable only of spectrographic or microchemical determination in the resultant alloys. After this they may be subjected to spectrographic or microchemical analysis in order to make sure that they are of the required degree of purity.

Any re-refining process that will bring about the desired substantial elimination of the impurities may be used. For instance, rhodium may be converted into a solution of rhodium chloride, precipitated from this as rhodium potassium nitrite and converted into rhodium potassium chloride, being recovered from a solution of this salt by reduction with formic acid. Platinum may be purified more simply, for example

by dissolving the metal in aqua regia and precipitating it as ammonium chloroplatinate.

The electrodes may be made from alloys containing other metals in addition to those mentioned. In particular the alloys may contain palladium, ruthenium, gold and silver, but these metals can be and normally are obtained commercially in a sufficiently pure state not to need re-refining. Moreover the alloys may contain base metals of high melting point, e. g. tungsten, molybdenum, copper and nickel, but in any case one or more precious metals predominate, that is to say, the predominating part of the alloy consists of precious metals although no single precious metal may amount to as much as 50% of the alloy.

I claim:

1. As an article of manufacture, a sparking plug electrode made from a member selected from the group consisting of the metals platinum, rhodium, iridium and osmium and alloys predominantly containing at least one of said metals, the predominant metal of said electrode being re-refined, and the said metal or alloy being so devoid of elements from the 25

group consisting of sulphur, selenium, tellurium, phosphorus, arsenic, antimony, bismuth, lead, tin, and silicon that the presence thereof cannot be determined with certainty by chemical analysis and that the total amount of elements from said group is less than 0.01%, said electrode being characterized by improved service life compared to a similar electrode containing elements of said group in excess of about 0.01%.

10 2. As an article of manufacture, a sparking plug electrode made from a member selected from the group consisting of the metals platinum, rhodium, iridium and osmium and alloys predominantly containing at least one of said 15 metals, the predominant metal of said electrode being re-refined, and the said metal or alloy being so devoid of elements from the group consisting of sulphur, selenium, tellurium, phosphorus, arsenic, antimony, bismuth, lead, tin and 20 silicon that the presence thereof cannot be determined with certainty by chemical analysis and that the total amount of elements from said group is less than 0.005%, said electrode being characterized by improved service life.

WILLIAM THOMAS GRIFFITHS.